

June 15, 1943.

G. W. BRANT

2,321,732

APPARATUS FOR EVAPORATIVE CASTING

Filed July 5, 1941



*Fig. 1*

*Gilbert W. Brant* INVENTOR

BY  
*Gilbert W. Brant*  
ATTORNEY

## UNITED STATES PATENT OFFICE

2,321,732

## APPARATUS FOR EVAPORATIVE CASTINGS

Gilbert W. Brant, Buffalo, N. Y., assignor to E. I. du Pont de Nemours & Company, Wilmington, Del., a corporation of Delaware

Application July 5, 1941, Serial No. 401,289

9 Claims. (Cl. 18—47)

This invention relates to evaporative (dry) casting apparatus, especially to the surface upon which the casting solution is spread, and comprehends the discovery that the common metal casting surfaces, when coated with sodium silicate, are rendered satisfactorily resistant to the chemical and physical actions normally encountered in the casting of thin sheeting of organic solvent soluble compounds.

The conventional details of evaporative casting involve the laying of a film of dope (solution of the material to be sheeted) on to a casting wheel or belt mounted for rotation and arranged for removal of the solvent from the dope during its rotation. The means for the solvent removal may include heating the casting surface or surfaces adjacent thereto, together with devices such as fans for carrying the solvent or solvent-laden atmosphere away from the film. Ordinarily the speed and degree of heating are adjusted so that the desired amount of solvent is removed in somewhat less than one revolution of the casting wheel or belt.

In dry casting, a film is formed which adheres relatively tenaciously to the casting surface. This cohesion, which is particularly tenacious in the case of some of the more common and potentially interesting sheet forming materials, has been the source of a number of direct and indirect difficulties. One of the principal difficulties is the pitting of the casting surface, due to the corrosive action of certain ingredients in the casting dope. As a result, it has been necessary to grind and buff, or otherwise refinish, metal casting surfaces at frequent intervals. Such refinishing are expensive and time consuming operations which very greatly increase the expense of the sheet material.

Improvements in the dry casting art, particularly reductions in the cost of refinishing metal casting surfaces, were the primary objects of this invention. How the foregoing objects and related ends are accomplished will be apparent from the following exposition, in which are disclosed the principle and divers embodiments of the invention, including the best mode contemplated for carrying out the same. The written description is amplified by the accompanying drawing, in which:

Figure 1 is a side elevation view partly in section, with some parts exaggerated in the interest of clarity, of a wheel casting device embodying the present invention; and

Figure 2 is a similar view of a portion of the

casting wheel with the relative dimensions of the parts somewhat out of proportion in order to better illustrate the details of the casting wheel. It has now been found that such objectives can be realized by applying the solution of sodium silicate to the metal casting surface and thereafter drying and baking the coating to render it hard, smooth and resistant to the action of organic solvents.

10 The most outstanding results have been obtained when the casting surface was made of stainless steel, copper or nickel. Improvements have also been obtained with other metallic surfaces such as iron, steel, nickel alloys and the like.

15 The metal surface should be uniformly smooth and preferably polished to a mirror-like finish and be carefully cleaned, especially if only a thin coating of sodium silicate is to be applied, before the coating operation.

20 Many varieties of sodium silicate are commercially available. They differ chiefly with respect to the ratio of the silica to the alkali, which may be anywhere from 1:1 to 4.2:1 or even higher.

25 This ratio affects the characteristics and properties of the dried coating, and it is therefore important in determining the sodium silicate to be used. The higher the ratio of  $\text{SiO}_2$  to  $\text{Na}_2\text{O}$ :

30 (1) The less easily the dried coating is dissolved or removed;

(2) The less the dried coating is affected by high humidity;

(3) The more brittle is the dried coating;

35 (4) The faster the coating dries with less retained water; and

(5) The less is the tendency of the coating to bloom.

40 If it is desired that the coating be easily removed, and if the casting surface is to be constantly maintained under atmospheric conditions of low humidity, a sodium silicate solution wherein the ratio of  $\text{SiO}_2$  to  $\text{Na}_2\text{O}$  is as low as 2:1, may be used with fairly good results. For most

45 purposes the ratio of  $\text{SiO}_2$  to  $\text{Na}_2\text{O}$  should not be less than 3.0:1, and where extreme brittleness and ease of removal are not important, as for instance, a more or less permanent coating on a casting wheel, the  $\text{SiO}_2$  to  $\text{Na}_2\text{O}$  ratio may be as high as 4.0:1 or even more. Because of its more

50 universal applicability, it has been found preferable to use sodium silicate solutions with  $\text{SiO}_2$  to  $\text{Na}_2\text{O}$  ratio in the range 3.0:1 to 3.6:1. Within this range coatings can be secured which are not so brittle as to be unsatisfactory on casting belts

(which are subjected to repeated bending in their course of travel) but which on the other hand are sufficiently hard and durable to provide a satisfactory casting surface over a long period of time.

The concentration of the aqueous sodium silicate (calculated as  $\text{SiO}_2 + \text{Na}_2\text{O}$ ) solution is important. In general, concentrations in the range 20% to 50% are satisfactory. The lower the alkalinity of the solution, that is, the higher the ratio of  $\text{SiO}_2$  to  $\text{Na}_2\text{O}$ , the more desirable it is to reduce the concentration. A concentration of 50% or even more may be used when the ratio of  $\text{SiO}_2$  to  $\text{Na}_2\text{O}$  is 2:1 or less. For ratios of 4:1 or more, the concentration should be in the neighborhood of 20% or even less.

The choice of a concentration is influenced somewhat by the method by which it is to be applied to the casting surface. As an example, a solution of sodium silicate wherein the ratio of  $\text{SiO}_2$  to  $\text{Na}_2\text{O}$  is 3.3:1 should have a concentration of about 25% to 30% for spray application, 30% to 35% for flow-on application, and 35% to 40% for spreading by means of a doctor knife or the like.

As previously indicated, the coating solution may be applied to the metal surface in any convenient manner. The more common schemes are spraying, flowing-on, dipping and spreading. When a plurality of thin coats are applied, as by spraying, each coat should be air dried before the subsequent coat is applied. Sodium silicate coatings, when subjected only to air drying, check or crack. Coatings which are force dried do not exhibit these undesirable characteristics, so it is essential that the air drying not proceed too far and that the coating be subjected to an elevated temperature while it contains a substantial amount of water. It is therefore advisable to carry out the several coatings in as short a time as possible. It has been found empirically that the time of air drying between coatings should not exceed about ten minutes at ordinary room temperature and ordinary normal or low room humidities. If the humidity is unusually high the time of drying (between coatings) may be prolonged.

If the sodium silicate coating is to be applied by flowing-on or dipping, time should be allowed for draining and to initially set the coating by air drying before a second coat is applied. A somewhat higher concentration of solution is used for this method of application, and as a result, the individual coatings are somewhat heavier. It follows that the number of coats may be considerably reduced except in those cases where a very heavy total coating is desired.

In those instances where a still more concentrated solution is applied and smoothed out by means of a doctor knife, a single application may be sufficient. Such a coating may be air dried until it is immobile, after which it should be subjected to force drying first at about 100° C. and subsequently at temperatures in the range 130°-150° C.

Because of the tendency of the coating to intumesce or froth, it is important that it not be subjected to excessively high temperatures while still hydrated to a considerable extent. These deleterious actions do not occur at 100° C. or 110° C. even when the coating contains a fairly high percentage of water. It is therefore generally desirable, when subjecting the coated surface to forced drying, to use an initial temperature of about 100° C. and gradually raise it to the range 140°-150° C. or even more. Excessive

drying should be prevented while the temperature is rising to 100° C., it having been found important that the coating still contain at least 25% water when it reaches this point. The coating should be heated soon enough and/or high enough to fuse it.

It is preferred that the final coating be a few thousandths (preferably five thousandths) of an inch thick. Any irregularities in the surface may be ground off and polished.

10 For convenience the invention has been described in terms of sodium silicate. It is to be understood that other alkaline (alkali metal) silicates, such as potassium silicate, may be used if desired.

15 The new coatings resist the action of the commonly employed neutral organic solvents such as acetone, toluene, ethyl alcohol, and those mentioned in the prior art patent cited earlier in the specification.

20 The alkaline silicate surfaces of this invention are useful in casting any of the types of organic solvent soluble self-sustaining coherent film forming materials. This includes the various

25 cellulose derivatives including the cellulose ethers such as methyl cellulose, ethyl cellulose, benzyl cellulose, ethyl benzyl cellulose and the like; cellulose esters such as cellulose acetate, cellulose propionate, cellulose butyrate, cellulose

30 aceto-propionate, cellulose aceto-butyrate, ethyl cellulose acetate, and the like; polyvinyl acetals such as polyvinyl formal, polyvinyl butyral and the like; vinyl resins such as vinyl acetate, vinyl chloride and the like; rubber derivatives such as

35 isomerized rubber, rubber hydrochloride, chlorinated rubber and the like, etc. It is especially useful in the casting of organic solvent soluble ethyl cellulose.

The new sodium silicate coatings are extremely 40 hard and smooth and show excellent adhesion to clean stainless steel, copper, and nickel surfaces. They form excellent bases for dry casting materials dissolved in organic liquids because inter alia they have high dielectric strength, low thermal conductivity, and permit ready stripping of water insoluble films, sheets and pellicles therefrom. Such pellicles are of uniform thickness and have smooth surfaces which are free from imperfections, blemishes, scratches, etc.

45 50 The properties of the sodium silicate coatings are such that they can be easily and quickly removed from the casting surface and economically renewed when desired. It is unnecessary to incorporate softeners or plasticizers in these coatings.

55 As many apparently widely different embodiments of this invention may be made without departing from the spirit and scope thereof, it is to be understood that this invention is not limited to the specific embodiments thereof 60 except as defined in the appended claims.

I claim:

1. A metallic casting surface from the group consisting of stainless steel, copper and nickel, having a thin coating of dried and baked alkali metal silicate.

65 2. A metallic casting surface from the group consisting of stainless steel, copper and nickel, having a thin coating of dried and baked sodium silicate.

70 3. A nickel casting wheel surface having a thin coating of dried and baked alkali metal silicate.

75 4. A nickel casting belt surface having a thin coating of dried and baked sodium silicate.

5. A metallic casting surface having a thin coating of dried and baked alkali metal silicate.

6. A metallic casting surface having a thin coating of dried and baked sodium silicate.

7. A metallic nickel casting surface having a thin coating of dried and baked sodium silicate, the ratio of  $\text{SiO}_2$  to  $\text{Na}_2\text{O}$  in the silicate being in the range 1:1 to 4.2:1.

8. A metallic nickel casting surface having a

thin coating of dried and baked sodium silicate, the ratio of  $\text{SiO}_2$  to  $\text{Na}_2\text{O}$  in the silicate being in the range 3:1 to 3.6:1.

9. A metallic nickel casting surface having a thin coating of dried and baked sodium silicate, the ratio of  $\text{SiO}_2$  to  $\text{Na}_2\text{O}$  in the silicate being 3:1.

GILBERT W. BRANT.

CERTIFICATE OF CORRECTION.

Patent No. 2,321,732.

June 15, 1943.

GILBERT W. BRANT.

It is hereby certified that error appears in the printed specification of the above numbered patent requiring correction as follows: Page 2, second column, line 5, for "head" read --heated--; and that the said Letters Patent should be read with this correction therein that the same may conform to the record of the case in the Patent Office.

Signed and sealed this 27th day of July, A. D. 1943.

(Seal)

Henry Van Arsdale,  
Acting Commissioner of Patents.